

April 11, 1939.

G. P. HOFF ET AL

2,154,204

RAYON STRUCTURES AND THEIR METHOD OF PREPARATION

Filed June 2, 1934

3 Sheets-Sheet 1



INVENTORS

BY GEORGE PRESTON HOFF  
HAROLD HENRY PARKER

*Charles F. Daley*  
ATTORNEY.

FIG. 1.

April 11, 1939.

G. P. HOFF ET AL

2,154,204

RAYON STRUCTURES AND THEIR METHOD OF PREPARATION

Filed June 2, 1934

3 Sheets-Sheet 2



FIG. 2.

INVENTORS

GEORGE PRESTON HOFF  
BY HAROLD HENRY PARKER

Charles F. Daley  
ATTORNEY.

April 11, 1939.

G. P. HOFF ET AL

2,154,204

RAYON STRUCTURES AND THEIR METHOD OF PREPARATION

Filed June 2, 1934

3 Sheets-Sheet 3



Fig. 3.



Fig. 6.



Fig. 4



Fig. 5

INVENTORS  
GEORGE PRESTON HOFF  
BY HAROLD HENRY PARKER  
Charles F. Daley  
ATTORNEY.

## UNITED STATES PATENT OFFICE

2,154,204

RAYON STRUCTURES AND THEIR METHOD  
OF PREPARATION

George Preston Hoff and Harold Henry Parker,  
Kenmore, N. Y., assignors, by mesne assignments,  
to E. I. du Pont de Nemours & Company,  
Wilmington, Del., a corporation of Delaware

Application June 2, 1934, Serial No. 728,862

3 Claims. (Cl. 57—157)

This invention relates to artificial yarn and particularly to the preparation of twisted structures such as strands and cords from strong artificial yarn of the regenerated cellulose type, and to their use in the manufacture of reinforced rubber articles such as rubber vehicle tires.

Strong rayon yarn is already known for use in reinforcing cord for rubber vehicle tires.

Cotton cord, commonly used in the manufacture of rubber vehicle tires, may be produced by twisting together five threads of 23 count cotton to about 20 turns per inch, then 3 strands thus formed are combined to form a cable by twisting them to 10 turns in a direction opposite to the strand twist. Such cord is commonly referred to as 23-5-3 construction. In making a comparable cord from strong rayon 5 threads of 275 denier-120 filament strong rayon twisted to 7 turns per inch are twisted together to about 20 turns per inch in a direction opposite to the twist of the threads. Three strands thus formed are then combined to form a cord by twisting them 10 turns per inch in a direction opposite to the strand twist and thus in the same direction as the thread twist. Such a cord will hereinafter be referred to as a 275-5-3 construction, the number 275 designating the thread denier; 5, the number of threads making up the strand; and 3, the number of strands in the cable. For the sake of facilitating a discussion of the invention, this construction is frequently referred to in the examples and throughout the specification, although it is to be understood that the invention is in no way limited thereto.

According to one known method of preparing a strong rayon cord of the above type, five 275-denier threads are led from a creel to the feed-in rolls by which they are delivered at a uniform rate. This bundle of threads, which is rapidly being twisted together, passes from the feed roll to a pigtail guide centered directly above the take-up spool and from it through the traveller on a ring, to the spool. The required twist, which may be 20 turns per inch right, is inserted during the thread travel from the feed rolls to the spool. Following this operation, three spools of the twisted strands are placed on a creel and the strands are twisted together in the reverse direction to about 10 turns per inch. However, if the doubling and twisting operation is conducted as above, the strands are characterized by marked irregularity of surface and the resulting cord has comparatively low strength.

In preparing cord from strong rayon, especially where the cord is to be used in reinforcing fabric

for rubber tires, it is frequently necessary to impart a high degree of twist, both while forming the intermediate strands, and also while plying the strands into the cord, in order that the cord may possess that degree of elongation and resilience essential to the efficient operation and long service life of the tires. Contrary to the experience and practice in the twisting of ordinary rayon and of cotton, the imparting of a high twist to strong rayon by conventional methods is accompanied by a great loss of strength (compared with what should reasonably be expected from the great initial strength of strong rayon), severe degradation of the thread, comparatively short service life, as well as other accompanying disadvantages. The marked difference between strong rayon and ordinary rayon, upon being given a high degree of twist, can be explained by the fact that the materials are essentially different in character. Thus, strong rayon has a strength per denier far in excess of ordinary rayon and its percentage elongation before failure is considerably less.

The following table sets forth the physical properties of an illustrative strong rayon thread and of a normal rayon thread:

|                         | Strong rayon<br>thread | Normal rayon<br>thread | 30 |
|-------------------------|------------------------|------------------------|----|
| Dry tenacity, g. p. d.  | 2.95                   | 1.64                   |    |
| Dry elongation, percent | 8.0                    | 21.5                   |    |
| Wet tenacity, g. p. d.  | 1.66                   | 0.82                   |    |
| Wet elongation, percent | 12.0                   | 30.8                   |    |

As further illustrative examples of strong rayon thread, we refer to those described in co-pending application of Harold H. Parker, Serial No. 676,463, filed June 19, 1933.

In view of the great potential importance of rayon cord and the like made from strong rayon, the disadvantages following from the practice of known methods for twisting strong rayon present a very serious problem to the art. The problem is particularly serious in view of the fact that strong rayon, due to its many valuable properties, offers considerable promise in the reinforcement of rubber tires and other reinforced rubber structures.

By way of illustrating the ineffectiveness of the methods now used for the twisting of strong rayon threads, when five 275 denier-120 filament strong rayon threads, having an initial twist of 7 turns per inch left, were plied and twisted together to 20 turns per inch right, and three such strands then plied and twisted together to 10

55

turns per inch left, according to known twisting methods, in order to obtain a cord to be used in reinforcing fabric for rubber tires, there occurred a strength loss which in many instances ran as high as 40%. This loss in strength is an indication of the extent of degradation of the threads during the twisting operation.

In accordance with the present invention, various methods of forming twisted rayon structures from strong rayon have been discovered which produced strands, cords, and the like, having tenacities, durability, service life, et cetera, greatly in excess of those obtainable by prior art methods, and having a smooth, uniform structure.

One object of this invention relates to the production of a twisted rayon structure possessing high tensile strength.

An additional object of this invention is to provide a rayon cord having high tensile strength and exceptional durability.

Another object of this invention is to provide a twisted structure formed of strong rayon in which the elements are uniformly spaced, and lie in place so that the resulting strand or cord possesses a high degree of uniformity.

A further object of this invention is to provide a method for twisting strong rayon on standard twisting machinery of the heavy duty type without substantially increasing the cost.

Another object of the invention relates to twisting of strong rayon yarn at a low relative humidity for the production of strong, uniform structures.

A still further object of the invention is the production of strong, uniform rayon strands and cords by a twisting operation in which twisting of an element is effected in a plurality of stages in the same direction.

Another object relates to the reinforcement of rubber structures, for example, rubber tires, by means of the strands and cords produced in accordance with this invention.

Other objects of the invention will appear from the description and the claims.

Referring to the drawings, Figure 1 represents a side elevation, partially in section, of a twisting machine adaptable for the practice of the invention. Figure 2 represents a front elevation, partially in section, of the same machine. Figure 3 is a side and detail view, partially in section, of some of the details of the machine. Figure 4 represents a detail view of a forming device which may be used in lieu of that shown in Figures 1 and 3. Figure 5 is a front view of a pulley comprising the forming device shown in Figure 4. Figure 6 is a magnified view of a strand twisted in accordance with the present invention.

In accordance with this invention, it has been discovered that a strand of even structure and high strength can be obtained without resorting to more than one operation by subjecting the thread during twisting to the action of a "forming" device comprising preferably a non-rotatable rod, but which may alternatively comprise a pulley, or any other equivalent appliance having a smooth surface, the forming device being placed between the twister feed rolls and the spool and over which the threads are drawn as they are twisted into a strand or cord. The forming device crowds the threads as they pass thereover evenly and uniformly around the center line of the finished strand or cord. Where a pulley is used as the forming device, it is preferably mounted so that it can rotate freely and can be driven by the motion of the strand. The use of such a

pulley minimizes the abrasive contact and is believed to have a definite beneficial shaping action on the bundle of threads as they roll or turn in the pulley groove while being twisted. The forming device may alternatively be a pulley which is directly driven from any suitable source of power, for example, by a frictional drive arrangement from the feed roll. In this modification, the amount of slippage is controlled by the effectiveness of the pulley drive and the relative sizes of feed roll and pulley.

In the carrying out of the invention, the position of the forming device in relation to the feed-in rolls is not a critical factor within reasonable limits. Thus, it may be placed in the same horizontal plane as the feed-in roll and 2" or 3" in front of the roll so that the bundle of threads passes from the forming device vertically downward to the spool. If desired, the forming device may be placed 8", 10", 12", or even 14" above the feed-in roll instead of in the same horizontal plane.

It is preferred, however, that the front portion of the periphery of the forming device be disposed directly above the spool so that the thread, after passing over the forming device, travels towards the guide which leads the thread on to the spool, in substantially a plumb direction.

Any standard make of down twister may be used in carrying out our process. The size of the twister, the speed of the spindles, the amount of twisting tension, or the particular design employed does not appear to alter the relationship between the results obtained with our improved method and those obtained by the previous method of twisting. While the relative results may thus be the same, it is preferable, in order to obtain the maximum strength to use twisters of the heavy duty type particularly designed for rubber vehicle tire cord work.

Where a non-rotatable rod is used as the forming device, we prefer to use a  $\frac{3}{4}$ " diameter rod although successful results may be obtained with  $\frac{1}{2}$ " diameter rods and with rods as large as 2" in diameter. Likewise, it does not appear that the diameter of the pulley, where a pulley is used as the forming device, is a critical factor since good results can be obtained with sizes, having a thread contacting periphery, ranging from  $\frac{3}{4}$ " to  $1\frac{1}{4}$ ".

Various materials of construction may be used for the rods or pulleys, for example, glass, porcelain, brass, steel, "Bakelite", or hard rubber. The rod or pulley should, of course, be smooth.

In the preferred embodiment of our invention, the use of a forming device of the character described has its greatest advantage in the twisting of the threads into strands. It can likewise be applied with advantage, however, to the cabling or cord-forming operation.

The following specific examples which refer to the drawings illustrate the use of a rod or a pulley as the forming device in the twisting operation:

*Example 1.*—Five threads 1 of 275 denier-120 filament strong rayon, having 7 turns initial twist left, and a dry strength of about 3 grams per denier at room temperature, are led downward from bobbins 2 mounted on a suitable creel 10, are gathered together on a convergence guide 16 and then fed by means of positively driven feed rolls 11 and 13 and frictionally driven intermediate roll 12 to the travelers 14 on ring 15 and wound onto suitably driven spools 17 with about 20 turns per inch right twist. A non-rotatable 7

glass rod 18, having a diameter of  $\frac{3}{4}$ ", is mounted by means of suitable brackets 20 which are adjustably fixed to standards 21, removably held in place on a supporting member 22. The rod 18 is positioned directly above conventional thread guides 23 and the spools, and is disposed parallel to and slightly above the feed-in rolls 11 and 13. The threads pass over rod 18 and are firmly held against it by the tension on the threads. Three 10 spools of strands 24 prepared in this manner are then taken and placed on the creel and are likewise twisted together on the same or on a similar twisting machine to give a final twist of 10 turns per inch, in a direction opposite to the twist in 15 the strand. The rod or other forming device need not be used during the twisting of the strands into cord. The cord prepared by this method possesses a dry tensile strength at room temperature of about 18 pounds, i. e. 1.68 grams 20 per denier, as determined by a Scott testing machine, as compared to a tensile strength of about 16.2 pounds, i. e. 1.44 grams per denier, for the best cord obtainable from strong rayon by prior art methods.

25 *Example II.*—The procedure is the same as for Example I except that instead of a rod, a plurality of axially aligned, freely rotatable pulleys 25, having  $1\frac{3}{4}$ " outside diameter and having  $1\frac{1}{4}$ " thread contacting diameter, are freely 30 mounted on a fixed rod 25 held in place in the same way as rod 18, as shown in Figure 4, and with the front extremity of the thread contacting periphery of the pulleys being disposed directly over thread guide 23.

35 *Example III.*—The procedure is the same as for Example I except that the single threads prior to being twisted into strands may have any twist up to 20 turns per inch.

40 *Example IV.*—In the previous examples, the direction of the strand or forming twist was the opposite of that of the initial twist in the thread. Our process may also be conducted to prepare a cord in which the first two twists, i. e., the thread twist and the strand twist, are in the same direction and the cable twist the reverse 45 of the preceding or strand twist. This type of construction is commonly referred to as the "hawser" type.

45 *Example V.*—The procedure is the same as for Example I except that the five threads making up the strand are twisted to 18 turns and the three strands are then twisted to 9 turns.

50 *Example VI.*—The procedure is the same as for Example I or II except that four threads instead of five are combined to make up the strand. Three strands are then twisted to form a cord. This construction is known as the 275-4-3 type. In this case, the strand twist is 23 turns instead of 20 and the cable twist upwards of 10.5 turns.

55 We find that strands prepared according to the processes of the above examples possess 10% 15%, and even 20% greater strength than is obtained by conventional processes. Likewise, cords prepared from such strands show upwards 60 of 20% increased strength with attendant increase in durability.

65 In addition to the increase in strength, the strands and cords prepared by the methods described above possess higher strength at elevated 70 temperatures. As an example, the strength of cords, prepared as described in the above examples, measured at 250° F., may be 16 pounds (1.42 grams per denier) or above, as compared to 13.7 pounds (1.21 grams per denier) for cord 75 made by a conventional process.

As a further improvement over known processes for twisting rayon filaments, thread, cords, and the like, in accordance with this invention, it has been discovered that the tendency of strong rayon, when given a high twist by previously known methods, (e. g., a twist of 18-22 turns per inch in the formation of a strand from 5 threads of 275 denier-120 filament strong rayon), to assume a rough, snarled appearance, can be overcome by carrying on the twisting operation in 10 two or more stages.

The following example illustrates a mode of applying this feature of the invention:

Example VII.—Five threads of 275 denier-120 filament strong rayon, having 7 turns left initial 15 twist and a dry strength at room temperature of about 3 grams per denier, are led downward from a suitable creel and then led by means of positively driven feed rolls through the traveler of a ring twister and are wound onto a spool with a 20 twist of about 10 turns per inch right. This operation is conducted in the same manner as regular ring twisting of cotton thread and standard equipment may be used throughout the process. The strand having 10 turns twist is then taken 25 and placed on the creel, and, in the same manner as the above, ten additional turns of twist are inserted in the same direction to give a final twist of 20 turns per inch right. The strand so prepared shows a strength at room temperature on a Scott tester of between 5 and 6 pounds (between 1.40 and 1.68 grams per denier) as compared to 3.5 to 4 pounds (0.98 to 1.12 grams per denier) which is the strength of a strand of 30 strong rayon which has been given its final twist 35 in a single conventional twisting operation.

The variations stated in Examples III to VI above may likewise be applied to the two-stage method of twisting with the same beneficial results obtained by the process of Example VII. 40 The multiple stage twisting operation may be effectively and conveniently carried out, however, in conjunction with the use of rollers or pulleys as "forming" devices as described in the preceding 45 part of this specification.

The prior art twisting of strong rayon threads results in a rough, snarled strand in which the threads do not lie evenly in the strand structure, some threads being more crowded than others and projecting above the surface of the strand. This is readily apparent from an inspection of a strand, magnified 25 diameters, and prepared in a single conventional twisting operation by imparting 20 turns right twist in a doubling operation to five threads of 275 denier-120 filament strong rayon having an initial twist of 7 turns left.

55 Referring to Figure 6 of the drawings, this figure represents a strand, magnified 25 diameters, prepared from five threads of strong rayon 60 yarn having seven turns initial left twist by first imparting to the threads 10 turns twist right, and then, in a separate twisting operation, imparting 10 additional turns right. Figure 6 clearly indicates the advantages to be derived by the 65 two-stage twisting operation of the present invention, the strand having an even, uniform structure and possessing a high strength and durability. The new strands furthermore possess a strength which may be 25%, 35% and even 70 50% higher than the prior art twisted strands, together with a far greater durability, length of service life, and resistance to failure, the uniformity of structure in the new strand permitting each element of the strand to sustain an 75

equal portion of the load at all times. Similarly, cords prepared from the new strands have correspondingly greater tenacity, service life, durability, resistance to failure, and when used as reinforcing fabric in rubber tires, eliminate blow-outs and other similar failures to a far greater extent than cords prepared from the prior art strands. Strands having satisfactory physical characteristics comparable to those of the strand shown in Figure 6, with a similar even, smooth surface, result from the use of the forming devices described in Examples I to VI, even where the twisting of the threads in the strand is accomplished in a single twisting operation.

The following table further illustrates the improvements realized by twisting strong rayon in the same direction in two or more stages, the letters "A" and "B" representing two types of strong rayon cord prepared by twisting three strands prepared as described in Example VII so as to form a cord having 10 turns in a direction opposite to the strand twist, the single twisting operation being designated as "one", representing the prior art twisting method:

| No. operations strand twisting | Scott tensile strength, pounds (at 70° F. and 60% relative humidity) |      |
|--------------------------------|----------------------------------------------------------------------|------|
|                                | A                                                                    | B    |
| One                            | 16.2                                                                 | 16.2 |
| Two                            | 17.6                                                                 | 18.8 |

The type of strong rayon thread designated "A" in the above table was formed from strong rayon filaments coagulated in the usual sulfuric acid-sodium sulfate coagulating bath. The type designated as "B" in the above table was formed from strong rayon filaments coagulated as described in co-pending application of Harold H. Parker, Serial No. 676,463, in a bath which contained zinc sulfate and glucose in addition to the usual sulfuric acid and sodium sulfate.

As explained above, it is usually desirable to twist the five threads of 275 denier yarn, which make up the strand, to about 20 turns per inch. It is to be noted that though the expression "20 turns per inch" has the appearance of a low twist, it is, in fact, a very high twist. The twist for different deniers required to produce a given strain in the thread varies indirectly with the denier. 20 turns per inch for five threads of 275 denier strong rayon yarn represent an extremely high twist for this type of yarn and result in a strand having a hard, compact structure. This hardness of structure makes it particularly necessary that the methods of this invention be used for high twist strands since in these cases, readjustment in position of the threads cannot readily take place once they are twisted together.

Our new two-stage twisting method produces strands and cords having improved hot strength as compared with prior art cords. Thus, cords prepared in accordance with the method of Example VII have a strength, measured at 250° F., of 17.4 pounds (1.54 grams per denier) as compared to 13.7 pounds (1.21 grams per denier) for strong rayon cords made by prior art methods.

This shows an increase of 26% in hot strength. All other tests used in the tire industry to evaluate cords for pneumatic tires, for example, fatigue and durability tests, show that cord prepared as described in Example VII, by the multiple twisting operation, is superior to previous cord

to an extent which may even be greater than would be expected to accompany the increase in tensile strength.

The twisting operations described in Examples I to VII are carried out at a relative humidity of above 60% and at a room temperature of about 75° F.

A major feature of this invention resides in the further discovery that when strong rayon threads are given a high degree of twist, if the twisting operation is carried out at a low relative humidity, that is to say, of less than 50%, a product is produced having a substantially higher cold and hot strength and a much greater uniformity and evenness of structure than where normal humidities, such as 65% and higher, are used, as in conventional twisting operations. This improvement is substantial even where ordinary single-stage twisting is used. The use of low relative humidity during twisting furthermore adds greatly to the improvement which follows from the use of forming devices such as rods or pulleys as is described in a preceding portion of this specification, or where the twisting of the threads into strands takes place in two or more twisting operations. The range of relative humidities used in order to get the best results will ordinarily be between 35% and 50%, although in some cases, relative humidities lower than 35% may be used. The temperatures maintained during twisting under low relative humidities will ordinarily range from about 75° to 95° F.

The following examples illustrate the use of low humidity in twisting operations:

*Example VIII.*—275 denier-120 filament regenerated cellulose thread having a dry strength of about 3 grams per denier, is finished in a suitable way with a solution containing about 1/2% of sodium oleate soap and twisted on a down-twister to 7 turns per inch left. Five of these threads are led downward from a suitable creel and then led by positively driven feed rolls to a traveler of a ring twister and onto a spool to give about 10 turns per inch right. A glass rod, having a diameter of approximately 3/4" is placed directly over the spool and under the thread parallel to and slightly above the feed-in rolls in the manner indicated in Figure 1 of the drawings. The threads pass over this rod and are held firmly against it by the twisting tension. This operation is conducted in the same manner as regular ring twisting of cotton thread, and standard equipment, other than the glass rod above noted, may be used throughout the process. The strands having 10 turns twist are then taken and placed on the creel, and, in the same manner as described in Example VII above, 10 additional turns or twists are inserted in the same direction to give a final twist of 20 turns right per inch.

The operation of Example VIII is carried out at a relative humidity of 45% and a temperature of 75° F. A strand prepared as described in this example has a strength on the Scott testing machine of between 5 and 6 pounds, as compared with strength of strands previously obtained of 3.5 to 4 pounds. Three of these strands are next twisted in a similar manner to 10 turns per inch in the reverse direction. The resulting cord has a dry strength at room temperature of over 21 pounds (1.85 grams per denier), as compared with previous cords having a strength of about 16 pounds (1.42 grams per denier). Furthermore, this cord has a hot strength of approximately 18 pounds (1.68 grams per denier), as compared with the maximum previously obtainable hot

strength of 13.7 pounds. It also has greatly improved durability and the smooth, uniform structure shown in Figure 6.

It is to be noted that in carrying out our invention in its preferred form, that is to say, with the use of low relative humidity, a number of improvements are combined, each of which contribute to the excellent result which is obtained. It is to be understood, of course, that it is not necessary to include each and every element mentioned heretofore to obtain results which are appreciably better than the results obtained by the prior art methods. To demonstrate this, we give below the following examples:

15. *Example IX.*—Five threads of 275 denier-120 filament strong rayon, which have not been twisted, are twisted to 7 turns on the customary rayon throwing machine. Five of these threads are then led downward from a suitable creel by means 20 of positively driven feed rolls and through a traveler of a ring twister onto a spool to give a twist of about 20 turns per inch, the twist being in the reverse direction to that of the elemental thread twist. Three strands so produced are then 25 doubled and twisted in the reverse direction in a similar manner to 10 turns per inch. All these operations are conducted on the standard down-twister of the heavy duty type such as is commonly used for twisting and doubling cotton thread.

30 The twisting is carried out at room temperature and at a relative humidity of 45%. The cord so obtained has a strength at room temperature of approximately 17.1 pounds (1.51 grams per denier) at 60% relative humidity and a hot 35 strength of approximately 15 pounds (1.33 grams per denier). It is to be noted that this mere change in humidity condition without the use of other improvements described throughout this specification improves the strength of the cord 40 at room temperature and also the hot strength, each in the neighborhood of 1 to 2 pounds, as compared with the results obtained when the relative humidity is 65% at room temperature as is customary in the twisting of rayon and cotton thread.

45. *Example X.*—The doubling and twisting operation is carried out as in Example IX on a twisting machine similar to that shown in Fig. 1 of the drawings and equipped with a  $\frac{3}{4}$ " glass rod. The cord so formed has a dry strength at room 50 temperature and a hot strength each about  $\frac{3}{4}$  lb. higher than the cord of Example I.

55. *Example XI.*—A twisting operation is carried out as described in Example IX with the exception that the intermediate strand twist is conducted in two stages as is described in Example VII. The cord so produced has a cold strength and a hot strength about equal to those of the cords produced in the previous example.

60. *Example XII.*—The process is carried out as in Example XI with the exception that the elementary threads are twisted on a down-twister to 7 turns per inch. An improvement of about one-half pound in cord strength is obtained.

65. The variations described in Examples III to VI may, of course, be applied to the low humidity twisting process referred to in the examples immediately preceding this paragraph.

70 While it is in general preferred to carry out the twisting operation at a relative humidity of 40-45%, it is desired to state that the lower the humidity, the greater is the tenacity of the twisted strand or cord. The relationship between decrease in humidity during twisting and increase in the tenacity of the cord is a straight

line function. This is illustrated in the following table which refers to a cord prepared by twisting 5 threads of 275 denier-120 filament strong rayon having a strength of about 3 grams per denier and having an initial twist of 7 turns left, into strands with 20 turns right, this operation being carried out in two stages, during each of which 10 turns is given the strands, three of the strands then being given 10 turns left in order to form the cord.

| Relative humidity | Dry tenacity in pounds at room temperature (Scott tensile test) |
|-------------------|-----------------------------------------------------------------|
| Per cent          |                                                                 |
| 45                | 18.7                                                            |
| 35                | 19.1                                                            |
| 24                | 19.5                                                            |

20 The foregoing examples quite clearly demonstrate the beneficial effect of the various features of the invention on the ultimate strength of the cords produced. The strand structures produced in accordance with Examples VIII to XII have substantially the same evenness of structure and appearance as the strand shown in Fig. 6 of the drawings, and are of the same general great utility.

25 Each of the methods of twisting described above, namely, twisting by the use of forming devices, multiple-stage twisting and twisting under low humidity conditions are susceptible of considerably variation. They may be applied to the twisting of threads of different denier than that specified in the examples, e. g. threads of a denier as low as 30, or as high as 1100, or even 1600 or higher, or the number of threads twisted into strands, or the number of strands twisted into cords may be varied. Likewise the number 30 of plying operations to produce the final product may be three or more, especially where low denier threads are used. Similarly, the new methods 35 may be applied to the twisting of threads having a low filament denier, e. g. 30 denier-30 filament, 120 denier-100 filament, 275 denier-250 filament, and other threads having a filament denier of the same order of magnitude. To indicate these 40 factors in an example not yet disclosed, our new method of twisting may be applied to the twisting of three threads of 450 denier strong rayon into a strand and then to the twisting of three of the strands into cord, with the same beneficial results 45 already described. They may be applied to the twisting of yarns obtained from different kinds of viscose, to the twisting of strong artificial yarn produced by the cuprammonium process, or of any other artificial yarn having physical characteristics comparable to those of strong rayon. While the processes described in this invention 50 are of most marked advantage in the case of strong rayon yarns having a low dry elongation, i. e. 12% or lower, at room temperature, strong rayon yarns having a high dry elongation, for example, 16%, can be twisted according to the 55 novel methods with advantage.

55 The amount of twist which is inserted in the various twisting operations may be varied, or the number of twisting steps in the multiple-twisting operation may be increased to 3 or more. The new twisting methods may likewise be used in conjunction with the various common devices, such as tensioning weights on the creel.

60 The twisting methods of the present invention 65 involving the use of "forming devices" or multiple 70

5

10

15

20

25

30

35

40

45

50

55

60

65

70

75

operation twisting may also be applied to the twisting of the threads while wet, e. g., after passing the threads through a water bath, as described in the co-pending application of Harold H. Parker, Serial No. 722,801, filed of even date herewith.

In the above methods for carrying out our invention, we prefer to use any suitable finish on the thread, and particularly prefer one which imparts to the thread a high degree of softness and slipperiness, e. g., soap, vegetable oil, or other lubricating material. As an example of a finish giving very satisfactory results, we may cite a solution containing simply about  $\frac{1}{2}\%$  of soap, calculated as sodium oleate. We find that the threads, when soaked in this solution and dried, have the desired characteristics which permit them to be readily twisted into smooth, even strand structures by our preferred process. Furthermore, the use of a finish substantially lessens degradation in the threads during twisting, and increases tenacity of the twisted structure.

The strong rayon referred to in the above examples and to which the twisting processes of this invention may be most beneficially applied, is prepared as described in co-pending application of Harold H. Parker, Serial No. 676,463, filed June 19, 1933, and has a strength of about 3 grams per denier. This thread is prepared by the use of a spinning bath containing zinc sulfate and glucose in addition to the usual sulfuric acid and sodium sulfate. While strong rayon prepared in this manner is preferred, any other strong rayon prepared by any other method, for example, by precipitating in the conventional sulfuric acid-sodium sulfate bath, may be used.

By the practice of this invention, there are produced strong rayon cords having a dry tenacity at room temperature of 18 pounds and higher, and having a hot strength of well above 15 pounds. These compare with maximum strength of about 16 pounds and about 13.7 pounds respectively obtainable under prior art methods. This invention may produce rayon cords having hot strengths substantially higher than those of the best grade Egyptian Sak cotton cord.

All the comparisons and discussions herein which refer to cotton relate to Egyptian Sak cotton which exhibits far superior characteristics when twisted into strands and cords than other types of cotton.

While the various improved results following from the practice of the invention have been described, for the most part, with reference to cords having a 275-5-3 construction and to the strands used in making up these cords, it will be understood that this construction has been chosen for the purpose of illustration and as a standard since it corresponds to the 23-5-3 cotton cord customarily used in the manufacture of pneumatic vehicle tires. The same relative beneficial results are obtained in applying the principles of the invention to the manufacture of strong rayon strands and cords which differ from the 275-5-3 construction in denier, number of filaments in the elemental threads, in the number of threads in the strands and in the number of strands in the cord. Thus, strands and cords varied in these various characteristics from the typical 275-5-3 construction, will, if produced in accordance with this invention, have a tenacity per denier of the same order as that of the 275-5-3 type.

It is noteworthy that not only do the various novel methods of twisting which constitute this invention improve maximum cord strength very

appreciably but they also have the further effect of decreasing the spread between maximum and minimum. Thus, for cord "A" of the table given on page 4, the maximum tenacity is 18.1 lb., and the minimum is 16.6 lb., and for cord "B", the maximum is 19.9 lb. and the minimum is 17.5 lb. This narrow spread between maximum and minimum, compared with a spread between maximum and minimum tenacities of prior art cords of some two to three times that of cords prepared by the twisting processes of the present invention, is very important since cord failures occur at points of minimum strength.

The term "room temperature" whenever referred to throughout the specification and claims is intended to be 75° F.

When the terms "elongation" and "percentage elongation" are referred to, they signify elongation at the breaking load.

It has been stated that the invention can be applied with great advantage to the production of rayon structures having a high twist. Thus, for example, in producing strong rayon cord for use in rubber tires, where the cord is to be of the 275-5-3 type, the intermediate strand may be given a twist of 20 turns per inch. It is to be noted that though the expression "20 turns per inch" has the appearance of a low twist, it is, in fact, a very high twist. The twist for different deniers required to produce a given strain in the thread varies indirectly with the denier. The most satisfactory method for determining whether a twist is a high twist or a low twist is by reference to the helix angle as defined in an article "An introduction to the micro-analysis of yarn twist" by E. R. Schwarz, published in the Journal of the Textile Institute for March, 1933, wherein it is stated on page 109:

"Barker and Midgley state, for example, that a Helix angle of 30° corresponds to a hard twist, and that a Helix angle of 45° represents normally an extremely high twist."

Using the equation developed by the above author, the helix angle for the strands prepared in accordance with the instant invention, i. e., 5 threads of 275 denier-120 filament, twisted to 20 turns per inch, is approximately 40°.

We have calculated the twist required for structures of different denier to produce this same helix angle. These values are summarized below:

*Twist to give same helix angle and therefore same degree of twist with structures of different denier*

| HELIX ANGLE, 40°             |                                           | 55 |
|------------------------------|-------------------------------------------|----|
| Denier                       | No. of turns per inch to give above angle |    |
| 100.....                     | 60.6                                      | 60 |
| 150.....                     | 49.4                                      |    |
| 275.....                     | 36.4                                      |    |
| 1050 (tire cord strand)..... | 20.0                                      |    |

Thus, it is seen that 20 turns per inch in a ply of five threads of 275 denier is in fact an extremely high twist.

The twisting methods of the present invention enable strong rayon yarn to be given a high degree of twist to produce a smooth, uniform surface with resulting increase in tenacity.

For the purposes of this invention, a high twist signifies a helix angle in the twisted structure, i. e. whether strand or cord, of above 35°, as determined by the equation referred to in said article.

The term "strong rayon", wherever used throughout the specification and claims, is intended to define rayon having a dry tenacity at ordinary room temperature of at least  $2\frac{1}{2}$  grams per denier. Throughout the specification, when reference is made to "strong rayon thread", without further qualification, it is to be understood that the thread has a twist of the order of 2 to 7 turns per inch. It is preferred that the strong thread have 7 turns per inch. It will be understood, however, that in some cases, this invention may be practiced with advantage with a strong rayon thread having no substantial twist.

In referring throughout the specification or claims to "dry thread strength at room temperature", or its equivalent, this is intended to indicate the tenacity obtained in the following manner:

The thread is reeled under uniform tension in 450-meter skeins; these skeins are conditioned for 3 hours in an atmosphere maintained at 60% relative humidity and 75° F.; the skeins are then weighed to determine the denier which is defined as the weight in grams of 9000 meters.

The tests for determining tenacity and elongation are made on a Suter single strand strength and elasticity tester with an oil plunger controlled pull. The rate of fall of the plunger is 1 foot per minute, and the distance between the clamps is adjusted for an 18-inch length of yarn. In making the dry test, five single strands from each of the above skeins are tested separately. These are clamped in the tester and stretched until the yarn breaks. Both the breaking load 35 in grams and the percent elongation may be read directly from scales on the machine.

Grams per denier are obtained by dividing the scale reading in grams by the denier of the thread.

The average of 50 dry breaks on threads selected at random is considered to be the tensile strength for any given 100-pound lot of yarn.

The dry strength of the strands or cords is obtained by conditioning at 60% relative humidity and 70° F. and testing according to the A. S. T. M. procedure D-179-30 (see A. S. T. M. Standard, vol. 2, 1930, page 1085).

The hot strength of cords given in this application are measured as follows:

A testing machine is provided with means for heating and maintaining the temperature of the cord during the tensile test at 250° F.; the cord is clamped between jaws initially 30 centimeters apart under an initial load of 4 ounces, and is then heated to 250° F.; when that temperature is reached, the cord is loaded at the rate of 10 lbs. per minute by means of water flowing through an orifice under a constant head into a bucket; the time to break the cord is measured with a stop-watch, and the breaking load is computed from this time, knowing the quantity of water that has flowed into the bucket. The initial load of 4 ounces is added to the measured load to give the total tensile strength of the cord in pounds.

Where methods of testing, other than those specifically referred to herein, are used, different numerical results may be obtained, but the relative improvement over the prior art will be of the same order, regardless of the method of testing used.

It will be readily understood from a study of the specification that by the practice of the various features of this invention, there are obtained rayon strands and rayon cords from strong rayon which have highly improved physical char-

acteristics, as compared with strong rayon twisted according to conventional twisting methods. Rayon strands, and more particularly rayon cords, produced according to this invention, are extremely useful as reinforcing means in the production of various articles which may or may not contain rubber. Thus, they may be used as reinforcing cord or fabric in rubber tires, in hose, in belts, such as fan belts or other power belts and conveyer belts, in loom harness, and generally in the manufacture of articles where it is desired to utilize the properties of the novel twisted structures. The high hot strength of our new strands and cords make them of particular value when used in reinforced articles which operate at a high temperature, such as pneumatic vehicle tires, steam hose, and conveyer belts used for the handling of hot materials. Rubber vehicle tires reinforced with the strands and cords prepared in accordance with this invention, as compared with tires reinforced with prior art cord, exhibit greater durability, longer service life, a lower rate of growth, a greater resistance to blow-outs, consume less power and thus lower the fuel consumption per mile, and operate at a lower temperature, since the tires reinforced with the new cords generate less heat, during the operation of the vehicle.

Any variation or modification which conforms to the spirit of the invention is intended to be included within the scope of the claims.

We claim:

1. A method of twisting strong rayon of the regenerated cellulose type and having a dry tenacity at ordinary room temperature of at least 2.5 grams per denier into a strand for use as a reinforcement for rubber structures which comprises imparting to the strong rayon a substantial twist and then, in a separate step, imparting an additional twist in the same direction. 40

2. The method of twisting strong rayon into a strand which comprises imparting a twist of about 2 to 7 turns per inch to threads of 275 denier-120 filament strong rayon, then twisting five threads in two steps to at least 18 turns per inch in the direction opposite to the twist of the threads. 45

3. A method of twisting strong rayon of the regenerated cellulose type and having a dry tenacity at ordinary room temperature of at least 2.5 grams per denier for use as a reinforcement for rubber structures which comprises producing a strand by imparting a substantial twist to a bundle of strong rayon threads and then, in a separate step, imparting additional twists in the same direction, and then twisting the resulting strand into a cord. 50

4. The method of twisting strong rayon which comprises producing a strand by imparting a twist of about 2 to 7 turns per inch to strong rayon threads of 275 denier-120 filament strong rayon, then twisting five threads in two steps to at least 18 turns per inch in the direction opposite to the twist of the threads, and then twisting the resulting strand into a cord. 60

5. The method of twisting strong rayon which comprises producing a strand by imparting a twist of about 2 to 7 turns per inch to strong rayon threads of 275 denier-120 filaments, then twisting five threads in two steps to at least 18 turns per inch in the direction opposite to the twist of the threads, and then twisting the resulting strand into a cord by imparting 9 turns per inch in the cord in a direction opposite to the strand twist. 70

6. The method of twisting strong rayon of the regenerated cellulose type and having a dry tenacity at ordinary room temperature of at least 2.5 grams per denier into a strand for use as a reinforcement for rubber structures which comprises imparting a substantial twist to a bundle of threads of strong rayon filaments, then further twisting the strand so formed by an additional twisting step in which the twist is in the same direction, further characterized in that the twist in at least one step is accompanied by a passage of the strand over a smooth curved surface disposed between the feed-rolls and the spool.
7. The process of twisting strong rayon threads of the regenerated cellulose type and having a dry tenacity at ordinary room temperature of at least 2.5 grams per denier into strands for use as a reinforcement for rubber structures which comprises carrying out the twisting op-

eration at a relative humidity of less than 50% and at a temperature of about 75-95° F., further characterized in that the twisting operation is carried out so as to give a twist in two successive stages in the same direction.

8. The process of twisting strong rayon threads of the regenerated cellulose type and having a dry tenacity at ordinary room temperature of at least 2.5 grams per denier into a strand for use as a reinforcement for rubber structures which comprises carrying out the twisting operation at a relative humidity of less than 50% and at a temperature of about 75-95° F., further characterized in that the twisting operation is carried out so as to give a twist in successive stages in the same direction, the strand during at least one of said stages being passed over a smooth curved surface.

GEORGE PRESTON HOFF.  
HAROLD HENRY PARKER. 20